

May 1, 1951

C. J. KINTNER ET AL

2,550,697

CLOTH WATER BAG

Filed May 8, 1946

2 Sheets-Sheet 1

Fig. 1.



INVENTORS  
Charles J. Kintner  
Wm. P. Hale  
BY  
Sigmund J. Lechner  
ATTORNEYS

May 1, 1951

C. J. KINTNER ET AL

2,550,697

CLOTH WATER BAG

Filed May 8, 1946

2 Sheets-Sheet 2

Fig. 2.



Fig. 3.



INVENTORS  
Charles J. Kintner  
BY Wm. P. Haar  
Sparta, New Jersey  
ATTORNEYS

## UNITED STATES PATENT OFFICE

2,550,697

## CLOTH WATER BAG

Charles J. Kintner, Birmingham Township, Chester County, Pa., and William P. Hall, Wilmington, Del., assignors to Joseph Bancroft & Sons Co., Wilmington, Del., a corporation of Delaware

Application May 8, 1946, Serial No. 668,258

7 Claims. (Cl. 28—78)

**1**  
This invention relates to water bags and a process for preparing cellulose fabric for the same.

It is general knowledge that cellulose fibers, whether natural, such as cotton and linen, or whether synthetic, such as viscose rayon, when subjected for a time to water, adsorb or absorb the water and swell beyond their normal size. This degree of swelling varies with the type of fiber, being, for example, less with cotton and greater with linen and viscose rayon.

It is also known that many materials exist which have the ability of imbibing water and of swelling excessively. Among such products we may mention, for example, gum arabic, gum tragacanth, gum karaya, alginates, methyl cellulose, polyvinyl alcohol. In fact, many substances which ordinarily are considered inactive toward water in this respect actually absorb water to a slight extent and swell, although sometimes this swelling is practically immeasurable. This phenomenon of slowly absorbing water has been used since early human times to cool drinking water beyond the temperature of the surrounding atmosphere. The ancients used goat skins and unglazed pottery jars, the latter being still in use.

The physical principles involved consist of evaporation of water from the outside of the moist bag or container into the surrounding atmosphere, the water evaporated being continually replaced by passage of water through the container wall. The latent heat of evaporation is furnished to some extent by the water in the bag and this removal of heat energy from the water results in a lowering of the temperature, thus producing water colder than the surrounding atmosphere. The rate of evaporation, and therefore the cooling effect, is to some extent, other factors being equal, dependent upon the surface available for evaporation, the greater the surface the greater the rate of evaporation. To obtain maximum cooling efficiency of a water bag, it is therefore necessary to have as large a surface as possible exposed to the atmosphere.

In the case of goat skins and earthenware jars, the container represents for all practical purposes a continuous surface, but if a woven cloth is used, the surface will consist of alternate yarns and interstices and will not be continuous and uniform as in a goat skin.

It is evident that the use of a woven cloth involves great difficulties since the water would tend to leak through the interstices, thus causing excessive leakage, making the bag impractical. Nevertheless, linen bags have been made which,

if tightly woven, work satisfactorily due to the marked swelling of the linen which gradually closes up the interstices until a satisfactory, slow passage of water is obtained. The linen bags, however, are costly as compared with a cotton bag, are susceptible to mildew and also are easily attacked by chemicals, such as the chlorine in purified drinking water.

Rayon might be used for this purpose, but, due to the poor wet strength of this material, it has not proven practical since great tensile forces will be applied to the cloth when the bag is full of water, this force being the greater the larger the bag.

**15** Cotton has been unsatisfactory for the purpose due to its low degree of swelling, the leakage occurring being excessive even when tightly woven fabrics are used.

To make use of cotton, manufacturers have resorted to the application of fabric sizing materials which, when in contact with water, will swell and prevent the excessive passage of water through the interstices. The materials used were those previously mentioned, such as, for example, gum tragacanth and methyl cellulose, employed in conjunction with a binder such as, for example, acrylate resins which act to retain or hold the swelling material and prevent it from loosening from the cloth and passing into the water. The plastic material in this case is an auxiliary material. However, impregnating the fabric with a sizing as described tends to close the fabric and to coat the individual fibers and yarns. By thus presenting a solid or continuous surface to the air, the cooling efficiency of the bag is decidedly less since the very large surface presented by the individual unsized fibers has been markedly reduced.

**40** We have now discovered that if certain cotton fabrics be treated as hereinafter described, water bags made therefrom meet the above requirements and in fact possess outstanding properties, better than heretofore obtainable.

Essentially, the discovery consists in partly altering such fabrics by chemical treatment, without destroying the fibrous and fabric nature of the material, so that when the cotton is brought into contact with water it will swell markedly and close up the interstices sufficiently to obtain the results without excessive leakage. In addition, the fabric prepared by this process has, as will be further shown, a relatively much larger surface for evaporation. The fabric has, by virtue of the treatment given, also acquired a valuable durable resistance to mildewing, and, in

addition, if desired, may have flame resistance.

To accomplish the desired objective, we select a fabric of the character hereinafter described and subject it to a mineral acid, and by chemical combination introduce acid groups into the cellulose by heating (i. e. curing) the treated fabric, at a temperature and for a time sufficient to bring about such chemical combination. The chemical which brings about the swelling being thus internally combined with the cellulose of the fibers, the evaporative surface of the fabric and of its yarns is retained unimpaired. Where, as in other processes, the fibers and yarns are coated, the evaporating surface of the fabric itself is reduced.

We prefer to use strong acids which will combine with the cellulose and which are not excessively volatile nor produce chemicals which will detrimentally alter the character of the fibers, under the conditions of the process, such, for example, as orthophosphoric, pyrophosphoric, sulfuric, polyphosphoric, orthophosphorous and pyrophosphorous acid, salts of said acids, substitution products of said acids and anhydrides of said acids.

The anhydrides, salts and substitution products of the acids should be capable of producing the proper pH condition on the cured fabric to insure combination with the cellulose and therefore volatile salts, such as ammonia and mono substituted polyacids, are recommended as these products will produce the proper conditions on the fabric.

Among substituted acids we may mention, for example, phosphamic, sulphamic, fluorophosphonic, phenylphosphoric and phenoldisulphonic acid.

It is possible to combine other acids such as, for example, phthalic, glutaric and salicylic acids by the above process but the swelling obtained with such acids is not of so high a degree. We, therefore, prefer to use the strong acids listed above (which by comparison are much stronger in their effect on the cellulose) and have obtained the most desirable results with ortho or pyrophosphoric acid with urea. Since those products are inexpensive and easily available they are recommended as the most practical in large scale production.

The acids should, as already stated, be capable of combining with the cellulose under the conditions of the process, and should not be excessively volatile nor decompose excessively under the conditions, should not extensively detrimentally alter the physical characteristics of the fabric, and should not introduce undesirable poisonous characteristics to the fabric.

The acid introduced imparts swelling, and mildew resistance. If the particular acid has flame-resistance imparting properties, this additional property also results. For example, orthophosphoric and sulfuric acids impart this property.

Since the acids are strong in nature it is desirable, for purposes of controlling the reaction, to introduce a nitrogen containing organic buffering agent or agents into the aqueous solution or mixture of the acid, said agent or agents to be present in sufficient quantities to produce a pH of from approximately 2 to approximately 7 on the cured cloth, the preferred range being from 3 to about 6, when tested with indicator solutions. By a buffering agent, we here mean such a substance or substances which will compete with the cellulose for the acid, thereby mini-

mizing the likelihood of objectionably tendering the material, particularly with respect to tensile strength. These substances are basic in nature, i. e., they are basic to the strong acid in solution.

Weak bases, such as urea, biuret, dicyandiamide, strong bases, such as guanidine, guanylurea, biguanide, and mixtures of strong and weak bases, may be employed. The weak bases are used in substantial excess as they do not sharply affect pH. Where a strong base is employed, i. e., one in which a change in quantity produces a marked change in acidity of the solution, it is desirable to use in addition a weak base such, for example, as urea and biuret. Other strong bases not of an organic character may be used to adjust the pH, i. e., reduce the acidity of the solution if too acid, such as, for example, soda ash, sodium hydroxide and borax, it being necessary in such cases to see that sufficient acid groups are available to insure combination with the cellulose and that sufficient buffering agent, such as urea, is present to prevent undesirable degradation of the cellulose. If the solution is slightly alkaline, the pH may be adjusted with an acid, such, for example, as acetic acid. The pH of the solution is usually higher than the pH of the cured fabric, ordinarily  $\frac{1}{2}$  pH higher or more. The general requirement of the pH of the solution is that it shall be such that the above set forth pH on the cured cloth is achieved during the curing. The pH usually drops during the curing.

Generally, we prefer a ratio by weight, of organic base to acid in the solution, of very roughly 2 to 1, but the ratio may vary widely as shown in the examples.

Insofar as a buffer is concerned, the general requirements are that it shall be such as to compete with the cellulose for the acid, shall be soluble to some extent in water and shall not cause objectionable degradation of the fabric, under the condition of the process.

Salts and substitution products of the bases mentioned above may be employed, provided they are of the general characteristics just described.

Where flame-resistance is also desired, the nitrogen incorporated due to the presence of the buffering base, supplements the flame-resistance imparting acid.

Although swelling of the fabric will be obtained when fabrics treated as above described are immersed in water, it is possible to obtain a great variance in this property. As will be shown, the conditions of the curing and also the chemical composition of the mixture on the cloth affect the results obtained. Thus, in Example 1, it will be shown that a formula using urea and orthophosphoric acid gives swelling which varies substantially with change in curing conditions, while, as shown in Example 2, a formula using urea, dicyandiamide, guanidine carbonate and orthophosphoric acid gives a swelling which varies comparatively little with change in curing conditions. The former formula when curing under the most suitable conditions, gives excellent swelling, while the latter gives relatively poor swelling under any condition, although practically the same type fabrics were employed.

Since the swelling tendency is a direct function of the quantity of water absorbed by the fibers, the difference in effect is apparently due to the smaller quantity of water absorbed by the latter complex. In the case of urea and orthophosphoric acid, the complex is more simple

than in the case of the urea, dicyandiamide, guanidine carbonate and orthophosphoric acid, the use of which results in more complex compounds.

Although the presence of a nitrogenous buffering agent is desired to control the reaction upon the cellulose, the presence of a large quantity of nitrogen in the finished fabric (the cured, washed fabric) is not essential unless substantial flame-resistance is also desired; in which case nitrogen in the complex is very useful. This is shown in Example 3, when a soaping with soda ash and soap removed nearly all of the nitrogen, leaving only a very small percentage. The resulting fabric, after coating, gave a very satisfactory water bag and the fabric itself had excellent swelling properties.

From the foregoing, it appears that the swelling property is to be attributed primarily to the acid groups in the complex, and, depending upon the bases employed, this property is affected very little or not at all where the base is urea and is reduced somewhat where mixtures of various bases are employed. In the former case, there is a combination which favors a maximum water absorption, while in the latter case the combination is less favorable. The resulting fabric, after coating, gave a very satisfactory water bag and the fabric itself had excellent swelling properties.

In the accompanying drawings, Figs. 1 and 2 are illustrative curves, the first of which is intended primarily to show the effect of time of cure and the second of which is intended primarily to show the effect of formulation and fabric.

Figure 3 is a simple conventional showing of a water bag made of the fabric of our invention and having a lid made of the same fabric.

Examples 1 and 2 also demonstrate the importance of the kind or construction of fabric which should be employed. In Example 1, an ordinary herringbone twill of about 8 ozs. to the sq. yd. was treated, and notwithstanding that the fibers showed marked swelling properties, the fabric was too loosely woven to make a really satisfactory water bag. The leakage is to great and the evaporating surface too small. On the other hand, in Example 2, the cloth is slightly heavier and somewhat better results would have been obtained had the formulation been more favorable to swelling.

The time and temperature of curing are very important and the degree of swelling is in part dependent upon these factors. The preferred time and temperatures are of course related to several factors such as the type of acid used, the pH on the cured fabric, the type of fabric and the nitrogenous buffering agent or agents used.

Generally, the lower the temperature the longer the time and the higher the temperature the shorter the time, other factors being equal. We prefer to use temperatures from 250° F. to 400° F. and time of cure from 120 minutes to 30 seconds, the preferred range being 300° F. to 350° F. and the preferred time from 8 minutes to 1 minute. Above these limits there is great danger that the fabric will be excessively degraded particularly with respect to strength. No satisfactory commercial results are obtained below these limits in reasonable time. It is to be understood that swelling takes place between wide limits in the time and temperature, as will be shown, but to get maximum swelling a definite condition is desirable during curing, other fac-

tors remaining the same. As an example, we may use urea and orthophosphoric acid, on herringbone twill (Example 1). We then find that a 2 minute cure gives moderate swelling; a 3 minute cure gives excellent swelling; and a 7 minute cure, poor swelling. This is shown by the curve of Figure 1. For each temperature, the curve will show a time peak, i. e., critical point, at which maximum swelling is obtained, and the time required to reach the peak will vary with the temperature, the lower the temperature the longer the time and vice versa. In Figure 2, the curve is relatively flat in comparison, but would still show a peak if the time of heating were extended. With any given set of conditions, it can readily be determined by test when the peak, i. e., maximum swelling is achieved. In this connection, it is to be observed that when imparting substantial flame-resistance as well as swelling, a similar curve for flame-resistance is obtained, but the flame-resistance curve and the swelling curve do not coincide. The peak of flame-resistance is achieved with a longer time of curing. In other words, maximum flame-resistance can only be achieved at some expense in swelling property, and best results, where both properties are desired, can only be had by compromise.

We prefer to use urea and orthophosphoric acid since these chemicals are inexpensive and easily available and give excellent results, and we prefer to cure the fabric as above described to get the maximum degree of swelling.

For the particular purpose of water bag fabrics, we prefer to use a heavy, tightly woven fabric as preventing objectionable leakage and as presenting adequate evaporating surface. We have obtained good results on certain cotton ducks, twills and oxfords of this general character.

Heavy, tightly woven fabrics such as, for example, hard texture or hard twist ducks from the #2/0 type to the #11 type weighing from 32 ozs. to 13 ozs. per square yard, also regular cotton duck from No. 3/0 to No. 11 weighing from 34 ozs. to 13 ozs. per square yard are suitable and have been used extensively in large scale production with results ranging from excellent to satisfactory.

We prefer the closely woven heavy type of fabrics (up to and inclusive of #10 duck) since they present a large evaporating surface to the atmosphere and therefore give greater cooling effect and when swollen prevent objectionable leakage. Other types of duck fabrics meeting the above specifications may be used with success, as may closely woven satins and twills of about 16 ozs. per square yard weight or heavier. It is evident that this process can also be applied to other cellulose fibrous materials such as, for example, linen and rayon, provided the weave or construction is about of the weight range given.

The best results are obtained with material comparable to #4 to #8 hard twist duck. The others mentioned may also be used, but it is desirable for optimum results to additionally treat the lighter weight fabrics as hereinafter pointed out.

In other types of finishes previously described, making use of a plain cotton fabric and sizes having water swelling properties, it is necessary to desize and scour the fabric to obtain the desired water absorbency. This is not the case with our invention where a grey unscoured fabric may be used to obtain good results, since the grey fabric after treatment has excellent absorbency.

We prefer, however, to have the cloth desized

and scoured to produce a good absorbent fabric prior to treatment. Mercerization, as stated, is beneficial and may be resorted to. The finish may be applied to undyed, dyed or printed fabrics, depending upon the effect desired.

The application of the solution follows conventional textile methods of application such as, for example, padding, printing and spraying. The fabric is then dried to remove the moisture and this is followed by the curing. The drying and curing may be combined into one operation. After curing the cloth may be given a washing to remove excess soluble chemicals.

Successive applications of size may be resorted to in order to obtain sufficient chemicals in the fabric. It is desirable, after the curing and washing, to have present in the fabric from approximately 8% to approximately 30% of chemicals. Higher solids take-on may be had but this does not appreciably improve the results, and lower take-on is apt to give unsatisfactory results. While the composition and the amount of chemical on the cloth is important, the concentration of the solution itself is unimportant, as either a single application or a succession of applications of the solution, with intermediate dryings, may be resorted to. In the case of a single application, with the squeeze set to give an approximately 100% solution pick up, the concentration should be such as to give an initial chemical take-on for the curing of from about 16% to 60% which would give an ultimate take-on in the cured, washed fabric from about 8% to about 30% as above indicated.

If the right cloth, say #4 hard twist duck, or its equivalent, is properly processed, a fabric may be obtained which will produce a satisfactory water bag, without further treatment, such as coating. It is, as previously indicated, beneficial in lighter weights, such as a #11 duck or similar weight cloth, or even somewhat heavier, to further treat by coating or impregnating the cured fabric, preferably the former, with a sizing solution to further reduce the passage of water through the bag. The sizing or coating mixture may be any material which will impede the passage of water through the fabric. We may mention, for example, waterproofing agents, waxes, plastics, resins and gums. We prefer to coat this water impeding material on one side (the inside) of the fabric since this procedure enables us to maintain a large surface on the outside of the bag and therefore, greater cooling efficiency. We may use film forming as well as swelling materials, such as, for example, vinylacetate-chloride copolymer, vinyl butyral, acrylate, polyethylene, rubber, polybutene, nitrocellulose, cellulose acetate, in fact, any of the textile coating materials well known in the art may be used as long as they impede the passage of water through the fabric and are not excessively water soluble. Some of these materials may be plasticized to obtain a satisfactory flexibility. Again, in this case the plasticizers used should not be excessively water soluble. They produce a discontinuous film, but nevertheless they reduce the size of the interstices by adding to the thickness of the yarn components of the fabric.

Materials which swell in water may be applied either alone or in conjunction with other materials, such as plastics. For example, methyl cellulose, polyvinyl-alcohol, gums, starch and alginates. The use of such swelling materials to impede the water is practical but not essential, since

if the proper fabric is used, sufficient swelling takes place in the fabric itself.

The great difference between our process and other processes now on the market lies in the fact that we obtain satisfactory results essentially by making the fabric swell in itself, while all other processes make use of sizing materials to cause the swelling while the fabric itself remains practically unaltered.

As previously stated, the alteration in the cellulose renders the fabric much less susceptible to attack by fungi and this is a very valuable aspect of the fabric. Since the chemicals are combined with the cellulose, they are not soluble in the cold water and, therefore, the mildew-resistance obtained is durable and without danger of poisoning so prevalent among the regular mildewproofing agents. Here, again, it is the acid and not the nitrogen in the finished goods which gives mildew-resistance. The fabric is also crease-resistant.

#### Example 1

To show the high degree of swelling obtained, a desized, scoured and dyed herringbone twill fabric (37", 72/46, 1.83 yds./lb.) having an original air porosity or air permeability of 7 seconds, when tested on the Gurley Densometer (using .10 sq. inch die, 5 oz. cylinder and 300 cc. of air) was impregnated (single application) with the following mixture:

400 parts urea  
200 parts orthophosphoric acid (75%)  
200 parts water

35  
800

followed by drying. Different sections were cured at different times, keeping the temperature constant at 320° F. After a thorough washing in hot water to remove all soluble material, the fabrics were dried. Samples of these fabrics were wet with water and then placed in a hydrostatic test machine and the time for the passage of 50 cc. of water was measured, this being again a measure of the degree of swelling. The longer the time the greater the swelling. The results given in the table below, and shown on the graph of Figure 1, show the phenomenal swelling of the treated fabric in water. An untreated fabric when placed in the machine allowed the water to pass through so rapidly (a few seconds) that no accurate measurement could be obtained.

| Time of Cure | Time for passage of 50 cc. Water |      |
|--------------|----------------------------------|------|
|              | Min.                             | Sec. |
| 2.0          |                                  | 54   |
| 3.0          |                                  | 101  |
| 3.5          |                                  | 81   |
| 4.0          |                                  | 33   |
| 4.5          |                                  | 23   |
| 5.0          |                                  | 17   |
| 7.0          |                                  | 11   |

55  
60  
65  
70  
75

The fabric used in this experiment is not well suited for water bags, but it serves to show the swelling effect obtained and illustrates how the peak, i. e., maximum swelling, can be readily ascertained.

It is evident that using this formula, fabric cured for a time sufficient to reach the highest point on the curve will be best suited for a water bag fabric.

The ratio of acid groups to pyranose units in

the cured, washed fabric, was about 1 to about 8 for the 3 minute cure, and about 1 to about 5 for the 7 minute cure. The sample cured for 7 minutes would be somewhat more flame-resistant, but would have somewhat less swelling property.

*Example 2*

To show the somewhat less degree of swelling obtained, when the chemical constitution of the mix is changed, a sample of 37% 88/56 1.32 yds./lb. desized, scoured and dyed twill fabric having an original air porosity or air permeability of 10 sec., when tested on the Gurley-Densometer (as described), was impregnated (single application) with the following mixture:

330 parts dicyandiamide  
750 parts urea  
70 parts guanidine carbonate  
500 parts orthophosphoric acid (75%)  
1050 parts water

2700

followed by drying. Different sections were cured at different times, keeping the temperature constant at 320° F. After thorough washing in hot water, the fabrics were dried. Samples of those fabrics were wet with water and placed in the hydrostatic machine and the time for the passage of 50 cc. of water noted. The results when compared with the previous example, indicate that despite the slightly denser cloth, the time was much less than before, thus showing that a smaller degree of swelling was obtained. The untreated cloth, however, allowed the passage of 50 cc. of water within 4 sec., proving that a definite swelling had taken place.

| Time of Cure | Time for passage of 50 cc. Water |
|--------------|----------------------------------|
| Min.         | Sec.                             |
| 1.0          | 26                               |
| 2.0          | 30                               |
| 3.0          | 30                               |
| 4.0          | 29                               |
| 5.0          | 30                               |
| 6.0          | 33                               |
| 7.0          | 31                               |
| 8.0          | 31                               |

The ratio of acid groups to pyranose units for the 3 minute cure was about 1 to about 9, and for the 7 minute cure was about 1 to about 5.

The results also show that with this formula the degree of swelling is not influenced as much by variance in time and that the more complex compounds produced do not favor water absorbency to the same extent as in Example 1.

*Example 3*

A scoured, dyed #6 hard twist duck was sized with the following mixture and dried:

390.0 parts polyphosphoric acid  
450.0 parts guanidine carbonate  
1500.0 parts urea  
3370.0 parts water

5710.0

The fabric was cured at 330° F. for 5 minutes, and then scoured in soap and soda ash followed by a thorough washing in hot water, and finally dried.

This fabric was coated on one side with:

100 parts acrylate resin emulsion (25% solid)  
25 parts 5% methyl cellulose solution  
4 parts ammonium hydroxide (28%)

and dried.

The water bags prepared from this fabric were excellent. Without the coating, the results are not as good.

*Example 4*

Scoured, bleached and dyed #6 hard twist duck fabric was impregnated thoroughly with a mixture of:

15 400 parts urea  
200 parts orthophosphoric acid (75%)  
200 parts water

800

20 followed by drying. The fabric was then cured 3 1/2 minutes at 330° F. and finally washed in hot water to remove all soluble material. The fabric was made into water bags without further treatment and found to serve satisfactorily.

*Example 5*

A regular cotton duck fabric weighing 15.20 ozs. per square yard was padded through:

500 parts fluorophosphoric acid  
1320 parts urea  
1000 parts water

2820 parts

dried, cured 4 minutes at 330° F. and finally washed to remove excess chemicals.

The fabric was then coated very lightly on one side with the following solution. An excellent water bag fabric was obtained.

40 19.0 parts Vinylite VYNW  
171.0 parts Vinylite VYNS  
147.0 parts Flexol D. O. P.  
45 240.0 parts methyl isobutyl ketone  
220.0 parts methyl ethyl ketone  
350.0 parts toluene

1147.0 parts

50 This demonstrates the use of a non-swelling coating, the closing of the fabric, being obtained entirely by the swelling of the fabric, the fibers or yarns of which have been somewhat increased in diameter by coating.

*Example 6*

A #8 hard twist duck previously scoured and dyed was treated with the following mixture:

60 300.0 parts conc. sulfuric acid  
750.0 parts urea  
750.0 parts water

65 dried and then cured at 340° F. for 3 minutes. After washing in hot water and drying, the fabric was coated on one side with the following emulsion:

70 65.0 parts polybutene  
104.0 parts Tervan 449 (wax)  
108.0 parts stearic acid  
104.0 parts methyl cellulose  
108.0 parts triethanol amine  
4588.0 parts toluene  
75 4334.0 parts water

## 11

The resulting fabric which demonstrates the use of a small quantity of swelling material (methyl cellulose) in the coating mixture gave a very good water bag.

## Example 7

A #4 hard twist duck, scoured to insure good absorbency, was impregnated with the following mixture:

|             |                      |
|-------------|----------------------|
| 100.0 parts | orthophosphoric acid |
| 65.0 parts  | dicyandiamide        |
| 75.0 parts  | acetamide            |
| 210.0 parts | water                |
| 450.0       |                      |
| 450.0 parts |                      |

dried and a portion then cured 4 minutes at 335° F., followed by washing in warm water. The results were excellent.

Another portion was coated on one side with a stearamidomethylpyridinium chloride wax emulsion prepared by mixing together:

|             |                                     |
|-------------|-------------------------------------|
| 100.0 parts | stearamidomethylpyridinium chloride |
| 12.5 parts  | guanidine carbonate                 |
| 11.2 parts  | acetic acid (70%)                   |
| 76.0 parts  | polyvinyl alcohol                   |
| 704.0 parts | water                               |

913.7

The resulting fabric gave exceptional results.

## Example 8

A secured and bleached #4 hard twist duck fabric was thoroughly impregnated with the following solution:

|           |                            |
|-----------|----------------------------|
| 300 parts | urea                       |
| 100 parts | biuret                     |
| 200 parts | orthophosphoric acid (75%) |
| 200 parts | water                      |
| 800 parts |                            |

followed by squeezing, drying and curing 3 minutes at 340° F. The cloth was then washed thoroughly in hot water to remove soluble materials and then dried.

Water bags made from this fabric were found to give excellent service.

## Example 9

A scoured and dyed #4 hard texture duck was impregnated with the following solution:

|             |                      |
|-------------|----------------------|
| 500.0 parts | urea                 |
| 500.0 parts | water                |
| 120.0 parts | fluorosulphonic acid |
| 1120.0      |                      |

and then dried.

One part of the fabric was curved 90 minutes at 250° F. and the second part 2 minutes at 400° F. After washing and drying the fabrics were given a light coat on one side with an acrylate resin emulsion. The resulting fabrics had good swelling properties and produced very satisfactory water bags.

## Example 10

A grey, unbleached and unscoured, regular #10 duck (15 ozs./yd.<sup>2</sup>) was thoroughly impregnated with the following solution:

|                         |                            |
|-------------------------|----------------------------|
| 200.0 parts             | orthophosphoric acid (75%) |
| 400.0 parts             | urea                       |
| Water to make 120 gals. |                            |

5  
10  
15  
20

and squeezed so that the solution pick-up was 100% by weight and then dried. The fabric was cured 4 minutes at 320° F. and washed in warm water, soaped in a dilute slightly alkaline soap solution, washed with water and dried.

The resulting fabric had excellent swelling properties and produced very good water bags without the application of sizing agents.

It will be seen from the foregoing that the weak bases, and more particularly urea, are to be preferred as interfering the least with the swelling effect imparted by the acid.

We have found that water bags made from cloth prepared as above described, work very satisfactorily under normal temperature and atmospheric conditions encountered over the United States and elsewhere, the rate of transpiration, i. e., of passage of water through the bag to the exterior, being for all practical purposes approximately equal to the rate of evaporation. Of course, under abnormal conditions such as at times of extreme relative humidity, the rate of evaporation will drop relatively.

The fabric of the invention suffers no objectionable loss of tensile strength from the treatment.

The #4 hard twist duck used had the following approximate specification: width 36", count 34/24, weight 24 ozs./yd.<sup>2</sup>.

The #6 hard twist duck had the following approximate specification: width 36", count 42/28, weight 20.5 ozs./yd.<sup>2</sup>.

The No. 10 regular duck had the following approximate specifications: width 36", count 45/32, weight 15 ozs./yd.<sup>2</sup>.

Another way of describing fabrics suitable for the purpose is by reference to air porosity and weight. Thus, for example, for initial cloth suitable for the purpose without any coating, an air porosity on the Gurley Densometer (under the conditions heretofore mentioned) of from 25 seconds and up, with a weight of from about 13 ozs. per sq. yd. and up, may be used, the higher the second value and the weight, the better the results. One may go to about as low as an air porosity of 10 seconds, with a weight of about 8 ozs. per sq. yd., where the coating is also employed.

In some cases it may be desirable, after the curing and washing, to impart a mechanical finish such as schreinering or calendering to make the fabric somewhat more dense. Similarly, especially where the fabrics are of the lighter weight and less dense construction, mechanical treatment such as schreinering can be advantageously employed after the curing and washing but before the coating is applied.

While we have indicated a solid concentration of 60% on the fabric to be cured, it will be understood that this may be exceeded, but the excess represents wastage as no material benefit result from the use of quantities in excess of 60%.

Using a solution formulation of phosphoric acid and urea for illustrative purposes, about the low limit of acid in the finished fabric in the washed state, for satisfactory results, is about 1 acid group to about 25 pyranose units. One may go much higher, in fact as high as possible, but extremely high ratios represent the use of unnecessary amounts of chemical without corresponding improvement in results.

We claim:

1. A water bag composed of cotton cloth having a construction and weight of the general order of those of #2 to #10 hard texture duck, and having acid groups chemically combined with the

75

cellulose in a ratio of not less than 1 acid group to 25 pyranose units, said cloth being characterized by a rate of transpiration approximately equal to the rate of evaporation, under atmospheric conditions ordinarily encountered, and by mildew-resistance and by a capacity for water swelling materially greater than that of cotton.

2. A water bag composed of cotton cloth having an air permeability ranging approximately from 25 seconds and up in the Gurley Densometer (using .10 sq. in. die, 5 oz. cylinder and 300 cc. of air) and a weight of from 13 ozs. and up per sq. yd., and having acid groups chemically combined with the cellulose in a ratio of not less than 1 acid group to 25 pyranose units, said cloth being characterized by a rate of transpiration approximately equal to the rate of evaporation, under atmospheric conditions ordinarily encountered, and by mildew-resistance and by a capacity for water swelling materially greater than that of cotton.

3. A water bag composed of cotton cloth having a construction and weight of the general order of those of #4 to #8 hard texture duck, and having nitrogen containing acid groups chemically combined with the cellulose with a ratio of not less than 1 acid group to 25 pyranose units, the said cloth being characterized by a rate of transpiration approximately equal to the rate of evaporation under atmospheric conditions ordinarily encountered, and by mildew-resistance and flame-resistance and by a capacity for water swelling materially greater than that of cotton.

4. A water bag composed of cotton cloth having a construction and weight not substantially less dense and lighter than those of #4 hard texture duck, and having acid groups chemically combined with the cellulose in a ratio of not less than 1 acid group to 25 pyranose units, said cloth being characterized by a rate of transpiration approximately equal to the rate of evaporation, under atmospheric conditions ordinarily encountered, and by mildew-resistance and by a capacity for water swelling materially greater than that of cotton.

5. A water bag composed of cotton cloth having a construction and weight of the general order of those of #2 to #11 hard texture duck, and having acid groups chemically combined with the cellulose in a ratio of not less than 1 acid group to 25 pyranose units, and the cloth being coated on one face with a discontinuous substantially non-water soluble coating and being characterized by a capacity for water swelling materially greater than that of cotton.

6. A water bag composed of cotton cloth having a construction and weight not substantially less dense and lighter than those of #10 hard

texture duck, and having acid groups chemically combined with the cellulose in a ratio of not less than 1 acid group to 25 pyranose units, said cloth being characterized by a rate of transpiration approximately equal to the rate of evaporation, under atmospheric conditions ordinarily encountered, and by mildew-resistance and by a capacity for water swelling materially greater than that of cotton.

7. A water bag composed of cotton cloth having a construction and weight of the general order of those of #2 to #10 hard texture duck and having acid groups chemically combined with the cellulose in a ratio of not less than 1 acid group to 25 pyranose units, said cloth being characterized by a rate of transpiration approximately equal to the rate of evaporation under atmospheric conditions ordinarily encountered and by mildew resistance and by a capacity for water swelling materially greater than that of cotton.

CHARLES J. KINTNER.  
WILLIAM P. HALL.

#### REFERENCES CITED

The following references are of record in the file of this patent:

#### UNITED STATES PATENTS

| Number    | Name             | Date          |
|-----------|------------------|---------------|
| 1,068,362 | O'Riely          | July 22, 1913 |
| 1,127,384 | Adams            | Feb. 9, 1915  |
| 2,012,159 | Eward            | Aug. 20, 1935 |
| 2,049,217 | Mennier          | July 28, 1936 |
| 2,089,697 | Sroebe           | Aug. 10, 1937 |
| 2,098,082 | Bowen et al.     | Nov. 2, 1937  |
| 2,099,363 | Heckert          | Nov. 16, 1937 |
| 2,174,534 | Shipp            | Oct. 3, 1939  |
| 2,225,589 | Haussmann et al. | Dec. 17, 1940 |
| 2,233,475 | Dreyfus          | Mar. 4, 1941  |
| 2,286,726 | Gordon           | June 16, 1942 |
| 2,302,107 | Dattow           | Nov. 17, 1942 |
| 2,332,047 | Bock et al.      | Oct. 19, 1943 |
| 2,401,440 | Thomas et al.    | June 4, 1946  |
| 2,467,792 | Wenzel et al.    | Apr. 19, 1949 |
| 2,504,124 | Hicks            | Apr. 18, 1950 |

#### FOREIGN PATENTS

| Number  | Country       | Date           |
|---------|---------------|----------------|
| 479,753 | Great Britain | Feb. 7, 1938   |
| 510,199 | Great Britain | July 28, 1939  |
| 547,846 | Great Britain | Sept. 15, 1942 |

#### OTHER REFERENCES

S. R. Merrill et al.: American Cotton Handbook, published by American Cotton Handbook Company (New York, 1941).  
Ser. No. 233,292, Schubert et al. (A. P. C.), published May 4, 1943.